

## UNITED STATES PATENT OFFICE

2,512,784

## LUBRICANT

David E. Adelson, Berkeley, Calif., assignor to  
Shell Development Company, San Francisco,  
Calif., a corporation of Delaware

No Drawing. Application December 26, 1946,  
Serial No. 718,617

12 Claims. (CL 252—48.2)

1

This invention relates to new and novel reaction products having properties of greatly improving and stabilizing lubricants. This invention also pertains to lubricants, such as mineral lubricating oils, synthetic lubricants of hydrocarbon and non-hydrocarbon origin, and the like, containing therein a multi-functional additive having detergent and anti-ringsticking properties, as well as acting as an inhibitor of oxidation and corrosion.

It is well known that various lubricants whether doped or undoped, tend to oxidize and to form corrosive bodies and sludge, when used in modern engines and machines operating under ordinary conditions or at high speeds, elevated temperatures, heavy loads and other adverse conditions. Some of the deterioration products of lubricants formed during their use are hard carbonaceous materials which adhere to metal surfaces and cause scratching and scuffing of movable metal parts and the sticking of valves and piston rings in engines. In addition, presently known lubricants are generally incapable of maintaining a continuous lubricating film between movable metal parts, resulting in gradual or rapid wearing away of metal parts. The damage thus caused required replacement of such parts or even the complete overhauling of engines and machines, resulting in expensive loss of production and time.

In the case of the highest quality non-corrosive, stable lubricating oils, highly refined for specific use, or synthetic lubricants developed for specific or special uses, it has been observed that such oils and lubricants are generally highly susceptible to oxidation and deterioration, becoming progressively more corrosive in engines and machines even under ordinary operating conditions.

To improve the lubricating properties of oils and synthetic lubricants it has become the practice to blend with various lubricants, one and in most cases more than one addition agents, which have the effect or property of inhibiting deterioration of lubricants and impart to them certain beneficial properties. Thus, additives have been specifically designed which have the property of inhibiting corrosion of alloyed bearings such as copper-lead, cadmium-silver and the like, developed for automotive, Diesel and aircraft engines. Acidic oxidation or decomposition components formed in lubricants during use readily attack these bearings but are inhibited or prevented from doing this by the formation of a corrosion protective film formed on the bearing surface with the aid of the additive. Additives have

also been developed which possess the property of modifying the carbonaceous materials formed, by deterioration of lubricants, on piston rods, rings and valves, and other metal parts in internal combustion engines, automotive and truck engines, aviation engines, high speed Diesel engines and the like. Such additives serve a very important function because, by modifying this carbonaceous material so that it can be removed easily, the tendency of engine parts to become stuck is inhibited so that ringsticking, piston scuffing, scratching and wearing away of other engine parts and material reduction of engine efficiency, are prevented or materially inhibited.

15 Other additives have been developed for the purpose of acting as detergents in lubricants in order to assist in the removal of soot or sludge, varnish, lacquer formed from deterioration of the oil when subjected to high operating temperatures. Detergents due to their cleaning action prevent the build up of these deleterious materials and assist in removing those formed. Anti-wear additives have the property of reducing friction of movable metal parts of the same or different metals. Due to the function exerted or property imparted by such additives on lubricants, wear caused by direct frictional contact of metals can be greatly reduced. Also, additives have been developed to withstand extreme pressures, disperse impurities, solubilize certain additives and the like.

The development of numerous additives has been due to the fact that an additive is capable of functioning in only one specific manner. Very few lubricant additives have the ability of improving a lubricant in more than just one respect. Thus, a good anti-oxidant might not be able to inhibit lacquer and varnish formation on piston rods or act as a detergent or corrosion inhibitor.

40 In many cases it is found that an additive possesses very good properties in one respect, but is the cause of harmful formations and therefore detrimental as an additive in another respect. Therefore, other additives are frequently required

45 to obtain a good stable lubricant. The combination of additives in lubricants wherein each additive exerts its influence without interfering with the function of other additives is a difficult matter to attain. In most cases additives co-react or interfere with each other. To prevent this great care must be taken in selecting the additives, mixing them in specific proportions and continuously watching and replacing additives which have stopped functioning or have deteriorated.

It is an object of this invention to improve the lubricating properties of various lubricating bases by the addition thereto of a minor amount of a multi-functional material. Another object of this invention is to add to compounded or doped lubricants a multi-functional material whereby a synergistic effect is produced, resulting in a product of accentuated and improved properties. Another object of this invention is to add to oleaginous materials, mineral lubricating oils, synthetic lubricants and the like, a multi-functional material so as to inhibit oxidation and corrosion and prevent the formation of sludge, varnish and lacquer in said lubricants even under adverse operating conditions. Still another object of this invention is to use in lubricating compositions, a multi-functional material which prevents ring-sticking as well as the sticking of other engine parts due to deterioration of the lubricant. Also it is an object of this invention to use in oleaginous materials, e. g. in lubricating compositions, a multi-functional material which inhibits wear, scuffing, scratching and other damage to engine parts. Furthermore it is an object of this invention to provide novel multi-functional improving and enhancing additives for lubricating bases. Other objects of this invention will appear as the description proceeds.

To the accomplishment of the foregoing and related ends, this invention consists of features which will be hereinafter fully described, and particularly pointed out in the claims, the following description setting forth in detail certain embodiments of the invention, these being illustrative of but a few variations in which the principles of the invention may be employed.

Basically, this invention contemplates the use in lubricants reaction products obtained by reacting organic compounds with hydrogen sulfide in presence of ammonium hydrosulfide. Among the organic compounds which can be reacted with hydrogen sulfide in the presence of ammonium hydrosulfide to produce oil additives of this invention are:

#### I. ALIPHATIC HYDROCARBONS

##### *Acyclic compounds*

A. Saturated paraffinic hydrocarbons above 6 carbon atoms such as

hexane  
heptane  
octane  
nonane  
tetradecane  
hexadecane  
eicosane  
tetracosane  
and the like.

B. Unsaturated paraffinic hydrocarbons above 6 carbon atoms such as

hexylene  
heptylene  
polyolefines  
which may be broadly termed polyalkenes, 65 and include polypropene, polypentenes as well as branched chain unsaturated hydrocarbons such as iso-olefines and iso-polyolefines.

##### *Cyclic compounds*

A. Saturated

cyclobutane  
cyclohexane  
cyclo-octane  
and the like.

B. Unsaturated

cyclopentadiene  
cyclohexene  
cyclo-octene  
and the like.

#### II. AROMATIC HYDROCARBONS

A. Benzene

Naphthalene  
Anthracene  
Phenanthrene  
Bi-phenyl  
Di-phenylmethane  
Stilbene  
and the like.

B. Alkyl

Hydroxy  
Amine  
Nitro  
Nitroso  
Halogen  
Carboxyl  
Mercaptan

Substituted aromatic compounds of group IIA and the like.

#### III. CYCLIC TERPENES

cymene  
limonene  
pinene  
bornylene  
methene  
terpinolene  
terpin  
menthol  
menthone  
isoborneol  
camphor

#### IV. HETEROCYCLIC COMPOUNDS

furan, furfural,  
furfuryl alcohol,  
furoic acid,  
pyrone, pyridine,  
picolinic acid,  
nicotinic acid,  
pyran, morpholine,  
coumarone  
and the like.

Both the cyclic terpenes and the heterocyclic compounds can have attached thereto substituent radicals, such as alkyl and alkenyl radicals, hydroxy and halogen groups, and the like.

#### V. ALCOHOLS

A. Aliphatic (saturated and unsaturated)

amyl alcohol  
hexyl alcohol  
heptyl alcohol  
octyl alcohol  
decyl alcohol  
dodecyl alcohol  
octadecyl alcohol  
carnaubyl alcohol  
oleyl alcohol  
Polyhydric aliphatic alcohols

glycols  
pinocols  
erythrol  
mannitol  
sorbitol  
and the like.

B. Aromatic alcohols  
 phenyl ethyl alcohol  
 phenyl octyl alcohol  
 octadecyl benzyl alcohol  
 benzyl alcohol  
 and the like.

C. Cyclic alcohols  
 naphthenic alcohol

D. Natural occurring alcohols and synthetic alcohols  
 Alcohols as found in wool fat, sperm oil  
 Alcohols produced by oxidation of hydrocarbons, e. g.

paraffin wax  
 sweat wax  
 petrolatum  
 and the like.

## VI. PHENOLIC COMPOUNDS

Phenol, alkyl phenol, catechol, resorcinol, pyrogallol.

All of these compounds may contain substituent groups such as alkyl radicals, amino, halogen, carboxyl and the like, hydroquinone, quinone, orcinol, phloroglucinol, cresols, thymol, saligenin, cinnamyl alcohol, methyl phenyl carbinol, eugenol, cardanols, etc.

## VII. ACIDS

A. Aliphatic (mono and polycarboxylic and hydroxy substituted acids and the like)

capric  
 undecyclic  
 lauric  
 myristic  
 palmitic  
 stearic  
 arachidic acids;  
 acrylic  
 sorbic, oleic, linoleic  
 linolinic acids;  
 hydroxy stearic  
 di and tri hydroxy stearic  
 ricinoleic acids;  
 alkyl malonic acid  
 alkyl succinic acid  
 alkyl glutaric acid  
 glycolic acid  
 pyruvic acid  
 phthalonic acid  
 lactic acid  
 alkyl maleic acid  
 alkyl malic acid  
 alkyl tartaric acid  
 alkyl citric acid  
 keto acids  
 suberic acid  
 alkyladipic acid  
 tartronic acid  
 and the like, acids produced by oxidation of hydrocarbon e. g.  
 paraffin wax and the like.

B. Aromatic acids

benzoic  
 salicyclic  
 cinnamic  
 hydrocinnamic  
 phthalic  
 naphthoic  
 abietic  
 naphthenic and sulfonic acids derived from petroleum hydrocarbons, mandelic acid, and the like;  
 phenyl acetic acid  
 phenyl stearic acid  
 naphthyl stearic acid  
 resinic acid

Both the aromatic and aliphatic acids of group VII can have attached thereto substituent groups as suggested under groups II, III, and IV.

## VIII. ESTERS

Esters contemplated for use in this invention may be obtained by reactioning any of the compounds listed under groups V and VI and their derivatives, with any of the acids listed under group VII.

## IX. ETHERS

The ethers contemplated for use in this invention may be symmetrical and unsymmetrical, or mixed ethers of dialkyl ethers, alkyl-aryl ethers, aryl ethers and the like. Specifically it is desirable to use:

### Ethers

A. Aliphatic (saturated and unsaturated)

20 methyl, ethyl methyl,  
 ethyl, ethyl propyl,  
 isopropyl, octyl,  
 ethers and the like;  
 vinyl, allyl, crotonyl  
 ethers and the like and mixture of saturated and unsaturated ethers.

B. Cyclic and poly ethers

ethylene oxide  
 propylene oxide  
 acetal, dioxan  
 and the like.

C. Aromatic ethers

35 anisole, phenetole,  
 diphenyl, dixenyl,  
 dinaphthyl ethers,  
 benzyl phenyl ether,  
 benzyl ether  
 cardanoxyethanol  
 and the like.

D. Substituted ethers

alkyloxy ethers of polyhydroxy aromatics such as resorcinol, pyrogallol, and the like.

## X. ALDEHYDES

A. Aliphatic (saturated and unsaturated)

45 acetaldehyde  
 propionaldehyde  
 butyraldehyde  
 caproaldehyde  
 and the like;  
 acrolein, crotonaldehyde, citral, etc.

B. Aromatic

55 Benzaldehyde  
 cinnamaldehyde  
 salicylaldehyde  
 naphthaldehyde  
 vanillin, etc.

## XI. KETONES

A. Aliphatic (saturated and unsaturated)

60 acetone, butanone, hexanone, oleone, palmitone, methyl ethyl ketone, methyl propyl ketone, butyrone, butenone, pentanone, phorone, pentanedione, mesityl oxide, diethyl ketone, 3-methylheptanone, di-isobutyl ketone, diacetone alcohol, and the like.

B. Aromatic

65 acetophenone  
 propiophenone  
 dibenzyl ketone  
 benzyl phenyl ketone  
 benzophenone  
 and the like.

## C. Cyclic ketones

Cyclobutanone  
cyclopentanone  
quinones  
cycloheptanone  
pure isophorone  
and isophorone bottoms the manufacture of  
which will be fully described hereinafter.

XII. NATURAL FATS, OILS AND WAXES AND  
THEIR DERIVATIVES AND MISCELLANEOUS COMPOUNDSA. Vegetable and animal oils, fats, and waxes  
such as:

castor oil  
coconut oil  
corn oil  
cottonseed oil  
horse fat  
lard oil  
mutton tallow  
beef tallow  
neat's-foot oil  
palm oil  
peanut oil  
rapeseed oil  
soya bean oil  
sperm oil  
whale oil  
wool fat  
Japan wax  
olefin waxes  
paraffin waxes  
wax tailings  
petrolatum  
vegetable and animal phosphatidic materials  
montan wax  
carnauba wax  
beeswax  
spermaceti  
castor oil distillate  
ozokerite  
tall oil, and the like

## B. Petroleum hydrocarbons such as:

naphtha  
mineral seal oil  
kerosene  
gas oils, etc.  
mineral oil

XIII. Metal salts and organic bases of organic acidic materials listed in any of the above groups, their mixtures, or various combinations may be treated with hydrogen sulfide in presence of ammonium hydrosulfide. Metal bases include those of the alkali metals, Cu, Mg, Ca, Cr, Br, Zn, Cd, Al, Sn, Pb, Cr, Mn, Fe, Ni, Co, etc. Organic bases include various nitrogen bases as primary, secondary, tertiary and quaternary amines.

Among the specific and preferred compounds contemplated for reacting with hydrogen sulfide in the presence of ammonium hydrosulfide may be mentioned: stilbene, oleic acid, ammonium oleate, potassium oleate, ammonium undecylenate, ethyl undecylenate, methyl ricinoleate, cottonseed oil, rapeseed oil, peanut oil, dehydrated castor oil, and tall oil as well as wax olefins, cinnamyl alcohol, pentanedione-2,4-diphenyl methane, high molecular weight saturated and unsaturated ketones, diacetone alcohol, mesityl oxide, ethyl oleate, ethyl cinnamate, cinnamaldehyde, and isophorone bottoms, the production and identification of which will be fully described below.

Isophorone bottoms are primarily high molecular weight unsaturated ketones having at least 12 and preferably more than 18 carbon atoms in the molecule. The synthesis of these products is obtained by condensation of acetone in caustic solution under elevated temperature and pressure. Specifically the product is obtained by condensing acetone in 30-60% caustic solution at a temperature ranging between about 10 130° C. and about 170° C. and under pressure of from 300 to 500 pounds per square inch. The resultant product is subjected to distillation to remove distillable ketones and other constituents and impurities. The product remaining in the 15 still is purified by filtration, solvent treatment and comprises of crude unsaturated cyclic ketones of high molecular weight, preferably referred to as crude isophorone bottoms. The term "isophorone bottoms" as referred herein is usually a 20 complex mixture of high molecular weight unsaturated cyclic ketones containing at least 12 and preferably more than 18 carbon atoms in the molecule. The product thus formed is not to be confused with straight isophorone which 25 is specifically 3,5,5-trimethyl cyclohexene-2-one-1, which is an unsaturated cyclic ketone containing only nine carbon atoms in the molecule. Isophorone bottoms produced by condensation of acetone under conditions referred to above 30 includes within its scope any and all unsaturated cyclic ketones containing at least 12 and preferably more than 18 carbon atoms and having generally the chemical structural configuration of isophorone as well as the chemical structural 35 configuration resulting from its condensation.

Crude isophorone bottoms can be fractionated and/or chemically treated and each fraction therefrom can in turn be treated with phosphorus sulfide at elevated temperatures to produce a 40 compound containing both phosphorus and sulfur. Among the various fractions which can be obtained from crude isophorone bottoms are topped, crude isophorone bottoms which contain at least 18 carbon atoms in the molecule and are obtained after removal of distillate from crude isophorone bottoms to a still head temperature of 45 140° C. at 10 mm. mercury pressure. Another fraction of crude isophorone bottoms can be subjected to hydrolysis with dilute sodium hydroxide and the acetone and isophorone formed removed by distillation. The bottoms can then be filtered and purified and comprise essentially unsaturated cyclic ketones containing at 50 least 12 and more carbon atoms in the molecule and are referred to as crude, hydrolyzed isophorone bottoms. This material can be subjected to distillation to split it into two fractions. The distilled hydrolyzed isophorone fraction has a boiling point of about 140° C. at 10 mm. mercury pressure and consists of a mixture of unsaturated 55 cyclic ketones containing between 15 to 18 carbon atoms in the molecule. The residue is referred to as topped, crude hydrolyzed isophorone bottoms and is similar to topped crude isophorone bottoms. They comprise essentially unsaturated cyclic ketones of at least 15 carbon atoms and higher in the molecule. Crude isophorone bottoms can be also subjected to condensation over 60 solid sodium hydroxide to yield two types of resinous materials. The first resinous fraction or soft resin has a viscosity at 210° F. of about 25-26 centistokes and an average molecular weight of from 320 to 350. The heavier fraction or medium resin has a viscosity at 210° F. of 65 about 25-26 centistokes and an average molecular

weight of from 320 to 350. The heavier fraction or medium resin has a viscosity at 210° F. of about 80 to 120 centistokes and an average molecular weight of from 370 to 390. All of the various unsaturated cyclic ketone fractions obtained in the manner fully described above can be used for reacting with hydrogen sulfide in the presence of ammonium hydrosulfide to form desired lubricating oil additives of this invention.

The reaction products of ammonium hydrosulfide-hydrogen sulfide with organic compounds can be prepared at room or elevated temperatures, preferably in enclosed vessels. No apparent advantage has been observed in using elevated temperatures to bring about the reaction except that it speeds up the reaction. However, the cost of fuel and special equipment outweighs this feature and it has been found more advantageous to simply allow the ammonium hydrosulfide-hydrogen sulfide organic compound reactions to take place at room temperature in enclosed vessels for at least one week to one month or more depending upon the organic material being treated.

To more clearly illustrate the present invention, the following examples are presented. It is to be understood however that various modifications can be resorted to without departing from the spirit of the invention as presented in the subjoined claims.

#### EXAMPLE I

Isopropyl alcohol (700 cc.) contained in a 4-liter, thick-walled suction flask, was saturated with dry ammonia followed by dry hydrogen sulfide. A solution of 238.5 grams of topped, crude isophorone bottoms in 350 cc. isopropyl alcohol was added and the resulting solution was saturated with hydrogen sulfide. The side-neck and mouth of the flask were then closed and the flask was allowed to stand for a week with infrequent shaking. Upon opening the flask a partial vacuum was discovered. The reaction mixture was filtered to remove impurities and the isopropyl alcohol was removed from the filtrate by evaporation. The residue was dissolved in 500 cc. of a non-aromatic hydrocarbon having a boiling range of between about 164° F. and 233° F. and washed with water. After removal of the solvent in a current of nitrogen gas on a steam bath, a very viscous sticky mass was obtained, said mass possessing a pleasant odor and exhibiting much less flow at room temperature than did the starting materials. The product was oil-soluble and on analysis contained:

|                                                                          | Analysis of Product | Analysis of cyclic ketone (topped, crude isophorone bottom) |
|--------------------------------------------------------------------------|---------------------|-------------------------------------------------------------|
| Percent by wt. Sulfur                                                    | 7.2 (5)             | 79.5 (9)                                                    |
| Percent by wt. Carbon                                                    | 76.2 (1)            | 9.8 (9)                                                     |
| Percent by wt. Hydrogen                                                  | 9.6 (2)             |                                                             |
| Percent by wt. Nitrogen                                                  | 0.26                |                                                             |
| Percent by wt. Oxygen (by difference)                                    | 6.6 (6)             | 10.5 (2)                                                    |
| Mol. wt. (ebulliscopic determination in C <sub>4</sub> H <sub>10</sub> ) | 352                 | 316                                                         |

#### EXAMPLE II

The same procedure was followed in this example as in Example I except that 243.5 grams of starting material was used and the reaction time

was one month. The analysis of the resultant product was as follows:

|                          |          |
|--------------------------|----------|
| Per cent by wt. sulfur   | 8.3 (7)  |
| Per cent by wt. carbon   | 75.7 (8) |
| Per cent by wt. hydrogen | 9.6 (1)  |
| Per cent by wt. nitrogen | 0.2 (7)  |
| Per cent by wt. oxygen   | 5.9 (7)  |
| Mol. wt.                 | 360      |

#### EXAMPLE III

The reaction with ammonium hydrosulfide-hydrogen sulfide in isopropyl alcohol medium (1315 cc.) was made with 295 gm. of topped, crude isophorone bottoms in an autoclave for 5½ hours at 96° C. to 101.5° C. The product was then treated as indicated in Example I and the analysis of the product was as follows:

|                          |          |
|--------------------------|----------|
| Per cent by wt. sulfur   | 6.2      |
| Per cent by wt. carbon   | 77.2 (3) |
| Per cent by wt. hydrogen | 9.6 (2)  |
| Per cent by wt. nitrogen | 0.3 (9)  |
| Per cent by wt. oxygen   | 6.5 (6)  |
| Mol. wt.                 | 356      |

#### EXAMPLE IV

Pure 3,5,5 trimethyl cyclohexene-2-one-1 was reacted with ammonium hydrosulfide-hydrogen sulfide as in Example I above and the analysis of the product was as follows:

|                          |          |
|--------------------------|----------|
| Per cent by wt. sulfur   | 26.4     |
| Per cent by wt. carbon   | 63.5 (5) |
| Per cent by wt. hydrogen | 8.9 (0)  |
| Per cent by wt. nitrogen | 0.2 (5)  |
| Per cent by wt. oxygen   | 0.9 (0)  |

#### EXAMPLE V

Ethyl oleate (53.6 gm.) was treated with ammonium hydrosulfide and hydrogen sulfide in isopropyl alcohol solution for one week and the desired product removed as indicated in Example I. The product on analysis contained 4.0% sulfur and proved to be an excellent rust and wear inhibitor.

Attempts have been made to determine whether any improvement in the reaction product could be attained by removing the air from the reaction vessel and carrying out the reaction in a hydrogen sulfide atmosphere or by continuously replenishing hydrogen sulfide at regular intervals. Reaction products carried out under such conditions indicated that no advantage is obtained and it has therefore been preferred to carry out the reactions as indicated in the illustrative examples.

Other ammonium hydrosulfide-hydrogen sulfide-organic compound reaction products which are particularly preferable as lubricating oil additives are as follows:

- 65 Ammonium hydrosulfide-hydrogen sulfide-mesityl oxide  
 Ammonium hydrosulfide-hydrogen sulfide-diacetone alcohol  
 70 Ammonium hydrosulfide-hydrogen sulfide-wax olefins  
 Ammonium hydrosulfide-hydrogen sulfide-stilbene  
 Ammonium hydrosulfide-hydrogen sulfide-pentandione-2,4

## 11

- Ammonium hydrosulfide-hydrogen sulfide-di-phenyl methane  
 Ammonium hydrosulfide-hydrogen sulfide-oleic acid  
 Ammonium hydrosulfide-hydrogen sulfide-ammonium oleate 5  
 Ammonium hydrosulfide-hydrogen sulfide-potassium oleate  
 Ammonium hydrosulfide-hydrogen sulfide-ammonium undecylenate 10  
 Ammonium hydrosulfide-hydrogen sulfide-ethyl undecylenate  
 Ammonium hydrosulfide-hydrogen sulfide-ethyl cinnamate  
 Ammonium hydrosulfide-hydrogen sulfide-methyl ricinoleate 15  
 Ammonium hydrosulfide-hydrogen sulfide-cottonseed oil  
 Ammonium hydrosulfide-hydrogen sulfide-rape-seed oil  
 Ammonium hydrosulfide-hydrogen sulfide-peanut oil 20  
 Ammonium hydrosulfide-hydrogen sulfide-dehydrated castor oil  
 Ammonium hydrosulfide-hydrogen sulfide-tall oil 25  
 Ammonium hydrosulfide-hydrogen sulfide-cinnamyl alcohol  
 Ammonium hydrosulfide-hydrogen sulfide-cinnamaldehyde

To illustrate the pronounced improvement obtained in lubricating compositions by the addition of small amounts of reaction products of this invention, the following test data are given:

TABLE I

## Oxidation stability determination

A refined undoped lubricating oil, 64-67 S. U. at 210° F. was employed, temperature 150° F.

| Additives                                                        | Catalyst: 1 cm. <sup>3</sup><br>Cu/gm. oil <sup>1</sup> |                              |
|------------------------------------------------------------------|---------------------------------------------------------|------------------------------|
|                                                                  | Amount per cent sulfate ash                             | 1,800 ml. oxygen time, hours |
| 1 None.....                                                      |                                                         | 7                            |
| 2 Ca petroleum sulfonate.....                                    | 0.3                                                     | 12                           |
| 3 Ca salt of alkyl phenol formaldehyde Condensation Product..... | 0.2                                                     | 18                           |
| 4 Ca petroleum sulfonate.....                                    | 0.1                                                     | 60.2                         |
| Reaction Product of Example I.....                               | 0.1                                                     |                              |

<sup>1</sup> All oxidation products corrected to 1,800 ml. oxygen absorbed per 100 g. of oil, assuming amount of product is proportioned to oxygen absorbed.

Additives of this invention were tested alone and compared with various lubricating oil additives in the multiple four-ball machine similar in principle to the Boerlage apparatus described in the magazine, Engineering, volume 136, July 14, 1933. This apparatus comprises four steel balls arranged in pyramid formation. The top ball is rotated by spindles against the three bottom balls which are clamped in a stationary ball holder. The balls are immersed in the oil to be tested. Tests were run two hours at 700 R. P. M. under 7 Kg. load and at a controlled temperature of 130° C. The diameters of the wear scars worn on the three balls forming the base of the pyramid were measured, and the average taken as the true indication of wear.

## 12

TABLE II

## Wear evaluation in the multiple four-ball machine

A refined undoped, lubricating oil, 64-67 S. U. at 210° F. was employed.

|                                      | Additive | Amount per cent sulfate ash | Scar diameter (mm.) at 7 Kg. load |
|--------------------------------------|----------|-----------------------------|-----------------------------------|
| 1 None.....                          |          |                             | 0.70                              |
| 2 Sulfurized wax olefin.....         |          | 0.1                         | 0.39                              |
| 3 Reaction Product of Example I..... |          | 0.1                         | 0.28                              |
| 4 Reaction Product of Example V..... |          | 0.1                         | 0.31                              |

The reaction products of this invention can be used as valuable constituents of heavy duty oils, motor oils, Diesel oils, aviation oils, turbine oil, synthetic oils and the like because of their anti-corrosion, antioxidation, and antiwear properties. The amount of additive used can be varied over wide limits but generally it is not necessary to use more than 5% by weight of the reaction product and preferably only between about 0.1 to 2.0% by weight is added to base lubricants.

Because of its synergistic effect the reaction product of this invention can be combined with other additives in lubricants, such as, blooming agents, pour point depressants or viscosity improvers, extreme pressure agents, antifoaming agents and the like. Among the specific additives which can be used are oil-soluble detergents which include oil-soluble salts of various bases with detergent forming acids. Such bases include metal as well as organic bases. Metallic bases include those of the alkali metals, Cu, Mg, Ca, Sr, Ba, Zn, Cd, Al, Sn, Pb, Cr, Mn, Fe, Ni, Co, etc. Organic bases include various nitrogen bases as primary, secondary, tertiary and quaternary amines.

Examples of detergent forming acids are the various fatty acids of, say, 10 to 30 carbon atoms, wool fat acids, paraffin wax acids (produced by oxidation of paraffin wax) chlorinated fatty acids, rosen acids, aromatic carboxylic acids including aromatic fatty acids, aromatic hydroxy fatty acids, paraffin wax benzoic acids, various alkyl salicylic acids, phthalic acid monoesters, aromatic keto acids, aromatic ether acids, diphenols as di-(alkylphenol) sulfides and disulfides, methylene bis alkylphenols; sulfonic acids such as may be produced by treatment of alkyl aryl hydrocarbons or high boiling petroleum oils with sulfuric acid; sulfuric acid mono-esters; phosphoric, arsenic and antimony acid mono and diesters, including the corresponding thio phosphoric, arsenic and antimony acids; phosphonic and arsenic acids and the like.

Additional detergents are the alkaline earth phosphate diesters, including the thiophosphate diester; the alkaline earth diphenolates, specifically the calcium and barium salts of diphenol mono and poly sulfides.

Non-metallic detergents include compounds such as the phosphatides such as lecithin and cephalin, certain fatty oils as rapeseed oils, volto-lized fatty or mineral oils and the like.

An excellent metallic detergent for the present purpose is the calcium salt of oil-soluble petroleum sulfonic acids. This may be present advantageously in the amount of about 0.025% to 0.2% sulfate ash. Also alkaline metal salts of alkyl phenol-aldehyde condensation reaction products are excellent detergents.

Antioxidants comprise several types, for example, alkyl phenols such as 2,4,6 trimethyl phenol, penta methyl-phenol, 2,4 dimethyl-6-tertiary-butyl phenol, 2,4-dimethyl-6-octyl phenol, 2,6-di-tertiary-butyl-4-methyl-phenol, 2,4,6 tri-tertiary-butyl phenol and the like; amino phenols as benzyl amino phenols; amines such as dibutyl-phenylene diamine, diphenyl amine, phenyl-beta-naphthylamine, phenyl - alpha - naphthylamine, dinaphthyl amine.

Corrosion inhibitors or anti-rusting compounds may also be present, such as dicarboxylic acids of 16 and more carbon atoms; alkali metal and alkaline earth salts of sulfonic acids and fatty acids; organic compounds containing an acidic radical in close proximity to a nitrile, nitro or nitroso group (e. g. alpha cyano stearic acid).

Extreme pressure agents which may be used comprise: esters or phosphorous acids such as triaryl, alkyl hydroxy aryl, or aralkyl phosphates, thiophosphates or phosphites and the like; neutral aromatic sulfur compounds of relatively high boiling temperatures such as diaryl sulfides, diaryl disulfides, alkyl aryl disulfides, e. g. diphenyl sulfide, diphenol sulfide, dicesol sulfide, dixylenol sulfide, methyl butyl diphenol sulfide, dibenzyl sulfide, corresponding di- and tri-sulfides, and the like; sulfurized fatty oils or esters of fatty acids and monohydric alcohols, e. g. sperm oil, jojoba oil, etc.; in which the sulfur is strongly bonded; sulfurized long chain olefins such as may be obtained by dihydrogenation or cracking of wax; sulfurized phosphorized fatty oils or acids, phosphorous acid esters having sulfurized organic radicals, such as esters of phosphoric or phosphorous acids with sulfurized hydroxy fatty acids; chlorinated hydrocarbons, such as chlorinated paraffin, aromatic hydrocarbons, terpenes, mineral lubricating oil, etc.; or chlorinated esters of fatty acids containing the chlorine in position other than alpha position.

Additional ingredients may comprise oil-soluble urea or thiourea derivatives, e. g. urethanes, allophanates, carbazides, carbazones, etc.; polyisobutylene polymers, unsaturated polymerized esters of fatty acids and monohydric alcohols and other high molecular weight oil-soluble compounds.

Depending upon the additive use and conditions under which it is used, the amount of additive used may vary from 0.01 to 2% or higher. However, substantial improvement is obtained by using amounts ranging from 0.1 to 0.5% in combination with phosphorous sulfide-unsaturated cyclic ketone reaction products of this invention.

It is to be understood that while the features of the invention have been described and illustrated in connection with certain specific examples, the invention, however, is not to be limited thereto or otherwise restricted, except by the prior art and the scope of the appended claims.

I claim as my invention:

1. A lubricant comprising a major proportion of a mineral lubricating oil and a minor amount, but sufficient to stabilize said mineral oil against deterioration and improve its anti-wear properties, of a stable, non-corrosive organic reaction product substantially free from nitrogen obtained by reacting for an extended period of time and at between about room temperature and about 100° C. ammonium hydrosulfide-hydrogen sulfide with an oxygen-containing organic compound until from 4% to about 26.4% sulfur enters the reaction product.

2. A lubricant comprising a major proportion of a mineral lubricating oil and a minor amount, but sufficient to stabilize said mineral oil against deterioration and improve its anti-wear properties, of a stable, non-corrosive organic reaction product substantially free from nitrogen obtained by reacting for an extended period of time at between about room temperature and about 100° C. ammonium hydrosulfide-hydrogen sulfide with 10 a ketone until from 4% to about 26.4% sulfur enters the reaction product.

3. A lubricant comprising a major proportion of a mineral lubricating oil and a minor amount, but sufficient to stabilize said mineral oil against deterioration and improve its anti-wear properties, or a stable, non-corrosive organic reaction product substantially free from nitrogen obtained by reacting for an extended period of time at between about room temperature and about 100° C. ammonium hydrosulfide-hydrogen sulfide with 15 an ester until from 4% to about 26.4% sulfur enters the reaction product.

4. A lubricant comprising a major proportion of a mineral lubricating oil and a minor amount, but sufficient to stabilize said mineral oil against deterioration and improve its anti-wear properties, of a stable, non-corrosive organic reaction product substantially free from nitrogen obtained by reacting, at between about room temperature and about 100° C. ammonium hydrosulfide-hydrogen sulfide with a salt of an organic acid until from 4% to about 26.4% sulfur enters the reaction product.

5. A lubricant comprising a major proportion of a mineral lubricating oil and a minor amount, but sufficient to stabilize said mineral oil against deterioration and improve its anti-wear properties, of a stable, non-corrosive organic reaction product substantially free from nitrogen obtained by reacting, at between about room temperature and about 100° C., ammonium hydrosulfide-hydrogen sulfide with an unsaturated cyclic ketone fraction having at least 12 or more carbon atoms and derived from condensation of acetone to 30 isophorone type fractions of high molecular weight until from 4% to about 26.4% sulfur enters the reaction product.

6. A lubricant comprising a major proportion of a mineral lubricating oil and a minor amount, but sufficient to stabilize said mineral oil against deterioration and improve its anti-wear properties, of a stable, non-corrosive organic reaction product substantially free from nitrogen obtained by reacting, for an extended period of time and at between about room temperature and about 100° C. ammonium hydrosulfide, hydrogen sulfide with ethyl oleate until from 4% to about 26.4% sulfur enters the reaction product.

7. A lubricant comprising a major proportion of a mineral lubricating oil and a minor amount, but sufficient to stabilize said mineral oil against deterioration and improve its anti-wear properties, of a stable, non-corrosive organic reaction product substantially free from nitrogen obtained by reacting, for an extended period of time and at between about room temperature and about 100° C. and in the presence of ammonium hydrosulfide, hydrogen sulfide with ammonium undecylenate until from 4% to about 26.4% sulfur enters the 55 reaction product.

8. A compound lubricant comprising a major proportion of a mineral lubricating oil and containing an active amount of calcium salt of alkyl phenol formaldehyde condensation reaction product, calcium salt of petroleum sulfonic acid as 70

## 15

detergents, and a small amount of an oil additive reaction product substantially free from nitrogen obtained by treating an oxygen-containing organic compound with ammonium hydrosulfide-hydrogen sulfide at between about room temperature and about 100° C. for a period ranging from between about 5 hours to over one month until from 4% to about 26.4% sulfur enters the reaction product.

9. A lubricant comprising a major proportion of a mineral lubricating oil and a minor amount, but sufficient to stabilize said mineral oil against deterioration and improve its anti-wear properties, of a stable, non-corrosive organic reaction product substantially free from nitrogen obtained by reacting, at between about room temperature and about 100° C., ammonium hydrosulfide-hydrogen sulfide with an unsaturated cyclic ketone fraction having at least 12 carbon atoms until said reaction product contains at least 6.2% sulfur and up to about 26.4% sulfur.

10. A lubricant comprising a major proportion of a mineral lubricating oil and a minor amount, but sufficient to stabilize said mineral oil against deterioration and improve its anti-wear properties, of a stable, non-corrosive organic reaction product substantially free from nitrogen obtained by reacting, at between about room temperature and about 100° C., ammonium hydrosulfide-hydrogen sulfide with ethyl oleate until said reaction product contains at least 4.0% sulfur and up to about 26.4% sulfur.

11. A lubricant comprising a major proportion of a mineral lubricating oil and a minor amount, but sufficient to stabilize said mineral oil against deterioration and improve its anti-wear properties, of a stable, non-corrosive organic reaction product substantially free from nitrogen obtained

5

15

20

25

30

35

## 16

by reacting, at between about room temperature and about 100° C., ammonium hydrosulfide-hydrogen sulfide with an oxygen-containing organic compound until said reaction product contains at least 4.0% sulfur and up to about 26.4% sulfur.

12. A lubricant comprising a major proportion of a mineral lubricating oil and a minor amount, but sufficient to stabilize said mineral oil against deterioration and improve its anti-wear properties of a stable non-corrosive organic reaction product substantially free from nitrogen obtained by reacting at between about room temperature and about 100° C., ammonium hydrosulfide-hydrogen sulfide with isophorone bottoms comprising essentially unsaturated cyclic ketone fractions having at least 18 carbon atoms in the molecule, until said reaction product contains at least 6.2% sulfur and up to about 26.4% sulfur.

DAVID E. ADELSON.

## REFERENCES CITED

The following references are of record in the file of this patent:

## UNITED STATES PATENTS

| Number    | Name     | Date          |
|-----------|----------|---------------|
| 2,230,691 | Lewis    | Feb. 4, 1941  |
| 2,279,560 | Dietrich | Apr. 14, 1942 |
| 2,413,648 | Ott      | Dec. 31, 1946 |
| 2,489,249 | Adelson  | Nov. 29, 1949 |

## OTHER REFERENCES

Organic Reactions, vol. 3, Adams, John Wiley, New York, 1946, chapter 2, pages 84, 92, 95, and 99 pertinent.

Inorganic Chemistry—Partington, MacMillan, 1926, page 800 pertinent.